

# UNITED STATES PATENT OFFICE.

MAX RÜPING, OF BERLIN, GERMANY, ASSIGNOR TO HULSBERG & CIE, M. B. H., OF CHARLOTTEBUEG, GERMANY, A LIMITED LIABILITY COMPANY OF GERMANY.

## IMPREGNATION OF WOOD, &c.

1,255,340.

Specification of Letters Patent.

Patented Feb. 5, 1918.

No Drawing. Application filed December 4, 1913, Serial No. 804,603. Renewed December 7, 1917. Serial No. 205,952.

*To all whom it may concern:*

Be it known that I, MAX RÜPING, a subject of the Emperor of Germany, residing at Berlin, Prussia, Germany, have invented 5 certain new and useful Improvements in Impregnation of Wood, &c., of which the following is a specification.

My invention relates in general to methods for preserving wood and similar materials, 10 and more particularly to impregnating the materials with preservative liquids.

My present invention has for its object to improve the method of preserving wood, and other materials, covered by U. S. Reissued 15 Letters Patent No. 12,707, dated October 22nd, 1907. In the practice of the method covered by the said reissued Letters Patent, the timber, or other material to be treated, is subjected to an air or gas pressure previous 20 to its immersion in the preserving liquid, the pressure being maintained and increased so that the pores, cells, and cavities in the material are first filled with air or gas of high pressure, which, after the material has 25 been thoroughly penetrated by the impregnating liquid, and the pressure has been released, expands and forces out of the material a portion of the preserving liquid. In the practice of the method covered by 30 my said patent, prior to my present invention, air has been exclusively used as the gas under pressure to which the material has been subjected in order that the excess preservative liquid may be expelled from the 35 material under treatment. The use of steam as the gas under pressure has heretofore not been considered feasible, inasmuch as the pressure of steam depends upon its temperature, and in most cases the material to be 40 treated, for instance wood, must not be subjected to a higher temperature than 240° F., and hence the available pressure of steam for this purpose is approximately 15 lbs., which is inadequate to satisfactorily secure the desired 45 results.

By my present invention the use of steam in the preservative treatment of wood, or other materials, is rendered possible by subjecting the wood to the successive combined 50 action of steam and air under pressure. The wood is first exposed to the action of steam up to a pressure of approximately 15 lbs.,

and when the steam pressure begins to exceed 15 lbs. the wood is subjected to compressed air, the wood, or other material under treatment, being of course inclosed within a receptacle into which first steam and air are admitted. The steam serves to heat and afterward moisten the cell walls so that they offer less friction to the passage into 60 the wood of the impregnating liquid, such as creosote oil. The reduction of the friction to the passage of the impregnating liquid through the cells and fibers of the wood, not only facilitates the permeation of the 65 wood by the liquid, but also expedites the ejection of the excess liquid by the expansion of the air inclosed in the individual pores and cells of the wood when the pressure around the same is released. In my improved method 70 the wood, or other material, is subjected to steam and air in succession before it is treated with the impregnating liquid, consequently the material is first heated and moistened by the steam at low pressure and 75 is then subjected to air at higher pressure than that of the steam.

In the practice of my improved method the wood or other material is inclosed within a retort and subjected to low pressure steam, 80 preferably not exceeding 15 lbs. to the square inch. Preferably before admitting the steam to the retort, a vacuum is created therein which renders it possible to use steam at lower pressure and promotes the rapid 85 penetration of the steam into the material.

While the material is still subjected to the action of the steam, compressed air of higher pressure than the steam is admitted into the retort and allowed to penetrate the material. 90 The compressed air entering the cells and pores of the material is moistened and heated by the steam and water of condensation which is formed in the retort and in the material as soon as air under pressure is admitted into the retort. The air distributes the steam condensed in the cells and pores of the material evenly throughout the entire mass thereof, thus rendering the material 95 more permeable to the preservative liquid and also imparting to the material such pliability that it will not split and check.

The steam outside the wood which has been brought to condensation by the air

pressure, and which has accumulated at the bottom of the retort is drawn off and the retort is then filled with the preservative liquid so as to entirely submerge the material therein. More of the preservative liquid is then forced into the retort, thereby increasing the pressure above that of the steam and air so as to force the preservative liquid into the material.

10 After the material has absorbed a sufficient quantity of the preservative liquid, the pressure is released to that of the atmosphere and the liquid is withdrawn from the retort. The compressed air confined in the 15 cells and pores of the material then expands with great force and expels the surplus preservative liquid from the pores of the material. The material is then preferably subjected to vacuum in order to evaporate the 20 water of condensation which has accumulated in the cells and pores of the material during treatment. The vacuum has the further effect of removing additional quantities of the preservative liquid from the material.

While in the preferred practice of my improved method the timber, or other material under treatment, should not be subjected to a vacuum after being steamed, as the steam 30 would thereby be expelled from the timber and the timber so cooled and dried as to impair the desired effect of the steam, yet if the timber under treatment has not been thoroughly seasoned it may prove advisable 35 to subject the timber to a vacuum after being steamed and prior to the subjection thereof to compressed air.

From the foregoing description it will be observed that I have invented an improved 40 method of impregnating wood or similar material with a preservative liquid, by the practice of which a better and more thorough distribution of the creosote oil, or other preservative liquid, is secured; the rapidity 45 of saturation is promoted; the necessary quantity of the preservative liquid is minimized; and the material under treatment is sterilized. These several advantages are primarily attained through the subjection 50 of the material to steam at comparatively low pressure prior to exposing the material to air or gas under a greater pressure.

I claim:-

1. The method of preserving wood and 55 similar materials, which consists in subjecting the material to steam, then subjecting the material to air or gas under pressure higher than that of the steam while the material is still subjected to the action of the steam, and then while maintaining the pressure around the material subjecting the same to an impregnating liquid under pressure.

2. The method of preserving wood and 65 similar materials, which consists in subject-

ing the material to steam, then subjecting the material to air or gas under pressure higher than that of the steam while the material is still subjected to the action of the steam, then while maintaining the pressure 70 around the material subjecting the same to an impregnating liquid under pressure, and finally relieving the pressure around the material and subjecting the same to a vacuum.

3. The method of preserving wood and similar materials, which consists first in subjecting the material to pressure below that of the atmosphere, then subjecting the material to steam, then subjecting the material 80 to air or gas under pressure higher than that of the steam while the material is still subjected to the action of the steam, and then while maintaining the pressure around the material subjecting the same to an im- 85 pregnating liquid under pressure.

4. The method of preserving wood and similar materials, which consists first in subjecting the material to pressure below that of the atmosphere, then subjecting the material to steam, then subjecting the material to air or gas under pressure higher than that of the steam while the material is still subjected to the action of the steam, then while maintaining the pressure around the material subjecting the same to an im- 90 pregnating liquid under pressure, and finally relieving the pressure around the material and subjecting the same to a vacuum.

5. The method of preserving wood and 100 similar materials, which consists in subjecting the material to steam at less than fifteen pounds pressure, then subjecting the material to air or gas under greater pressure than the pressure of the steam while the material 105 is still subjected to the action of the steam, and then while maintaining the pressure around the material subjecting the same to an impregnating liquid under still greater pressure.

6. The method of preserving wood and similar materials, which consists in subjecting the material to steam at less than fifteen pounds pressure, then subjecting the material to air or gas under greater pressure than the pressure of the steam while the material is still subjected to the action of the steam, then while maintaining the pressure around the material subjecting the same to an im- 115 pregnating liquid under still greater pressure, and finally relieving the pressure around the material and subjecting the same to a vacuum.

7. The method of preserving wood and similar materials, which consists in first sub- 125 jecting the material to pressure below that of the atmosphere, then subjecting the material to steam at less than fifteen pounds pressure, then subjecting the material to air or gas under greater pressure than that of 130

the steam while the material is still subjected to the action of the steam, then while maintaining the pressure around the material subjecting the same to an impregnating liquid under still greater pressure, and finally relieving the pressure around the material and subjecting the same to a vacuum.

In testimony whereof, I have subscribed my name.

MAX RÜPING.

Witnesses:

HENRY HASPER,  
WOLDEMAR HAUPT.